

2,828,194

## ETCHING

Charles W. Hopkins and John A. Easley, Midland, Mich.,  
assignors to The Dow Chemical Company, Midland,  
Mich., a corporation of Delaware

No Drawing. Application September 28, 1956  
Serial No. 612,886

10 Claims. (Cl. 41—43)

This invention relates to a method for etching the surface of a metal object, and is more particularly concerned with an improved method and bath for etching photoengraving plates.

In the conventional method of making a metal printing surface, such as a photoengraving, a plate of an acid-soluble metal such as magnesium, zinc, or one of their alloys is firstly coated with a light-sensitive coating or "enamel," applied to the generally flat or cylindrical metal surface. This coated surface is then exposed to light through a negative having an image thereon so as to produce a corresponding image on the coating. The exposed coated surface is then "developed," forming an acid-resistant coating in the form of the image produced by the exposure. This acid-resistant coating is further hardened by heating and the image-bearing surface of the plate is then subjected to etching by an acid. In prior art techniques, as the etching proceeds, the acid tends to etch laterally and thereby undercut the resist, causing a weakening or a distorting of the image. While art techniques have proposed to prevent or reduce the amount of undercutting by repeatedly "powdering" the plate, and partially etching between each powdering application, this has been a time-consuming and difficult operation.

It is a principal object of the present invention to provide an improved method for etching metal and particularly photoengraving plates. Another object of the present invention is the provision of etching baths for carrying out the improved process for etching. Still a further object of the present invention is to provide etching baths containing particular sulfated materials, e. g., sulfated fats, oils and/or waxes. Another object of the present invention is the provision of such etching baths containing particular amounts of the above materials. Other objects will become apparent hereinafter.

This invention is directed to an etching technique which may be accomplished by providing an etching bath containing aqueous nitric acid, an immiscible organic liquid substantially unreactive with the aqueous nitric acid solution, and a water-soluble, anionic, surface-active half ester of sulfuric acid, containing at least one hydrophobic group therein, said hydrophobic group containing between 10 and 26 carbon atoms in an uninterrupted chain, said ester also containing at least 8 percent sulfation, the ester usually being derived from the sulfuric acid treatment of naturally-occurring fats, oils and waxes.

Suitable metals which may be etched by the process and bath of the present invention are magnesium, magnesium base alloys containing at least 85 percent magnesium, and zinc and zinc base alloys containing at least 90 percent zinc. To prepare a photoengraving plate, the surface of the metal is first coated uniformly with a light-sensitive material, exposed to light through a negative, developed, and, if necessary, heated to increase the acid resistance of the resist. When the plate to be etched has been so treated, it is then ready for use in the method of the present invention.

Aqueous nitric acid for the bath of the present invention is employed in an amount by weight of the total bath between about 1 and 25 percent  $\text{HNO}_3$ , concentrations in the range of from 3 to 20 percent  $\text{HNO}_3$  being most generally useful, while a concentration of from 4 to 12.5 percent is preferred. The aqueous nitric acid is mixed with a water-immiscible organic material which is liquid at those temperatures employed for etching. This organic liquid should also be substantially unreactive with the aqueous nitric acid solution. Suitable organic materials which may be used in the method and bath of the present invention include, for example, the various petroleum fractions boiling in the range of 70° to 390° C., such as gasoline, benzene, kerosene, coal oil, and lubricating oils. Other organic liquids which may be employed include turpentine, perchloroethylene, the diethylbenzenes, tetramethylbenzenes, isopropylbenzene, carbon tetrachloride, etc. The amount of organic liquid employed will vary with the type of metal surface to be processed, but will fall within the range of 1 to 12 percent by weight of the total bath and preferably is from 5 to 8 percent.

A third component of the bath, e. g., a sulfated fat oil or wax, includes a sulfate-radical-containing, organic surface-active agent. This component can further be described as containing at least in part a half ester of sulfuric acid, the component being water-soluble, anionic, and containing at least 8 percent sulfation, preferably at least 14 percent. Percentage of sulfation, as used herein, is intended to mean the average amount of sulfate ( $\text{SO}_4$ ) contained in the molecule divided by the practical amount of sulfation possible multiplied by one hundred. The hydrophobic portion of the surface-active agent must contain at least one aliphatic organic group containing at least 10 carbon atoms and not more than 26 carbon atoms, and preferably from 14 to 26 carbon atoms. Suitable sulfated materials which may be used in the bath of the present invention include, for example, sulphated tall oil, sulfated castor oil, sulfated sperm oil, sulfated tallow, sulfated propylene, alkylarylpolyether sulfates, sulfated amides, sulfated alcohols, the monoglyceride ester of coconut oil sulfate, etc. These materials are generally available commercially under various trade names. It has been found that the amount of the third component employed is critical, the effective range of concentration being between 0.4 and 2.0 percent by weight of a total etching bath. For example, Monosulph (Nopco Chemical Company—a sulfated castor oil having 45 percent sulfation containing 30 percent water, 2 percent sodium sulfate, 24 percent sulfated ester, 28 percent unreacted neutral oil and 16 percent sulfated acids and soap and free fatty acids) has an optimum effective concentration of 1.16 percent.

In practicing the present invention it has been found to be desirable to impinge the bath against the surface to be etched, as by splashing. In theory, at least, the etching bath of the present invention forms a partially acid-resistant film on the resist-free metal surfaces, and when the bath is impinged against the surface to be etched in a direction normal to that surface, the film is broken. On the other hand, when the bath hits the sides of the relief the film is generally not broken because of insufficient striking force and etching of the sides (or undercutting) is substantially reduced. It is preferred to employ an etching machine of the type disclosed in Patent No. 2,669,048, issued February 16, 1954, and entitled "Etching Machine." In this machine elongated paddles dipping into the bath composition intermittently throw, by splashing, the etching bath composition in sheets upwardly against the image bearing side of the object being etched, e. g. a plate.

As used in this specification, the term "etch factor," is defined as the ratio of the depth of the etch adjacent to a line of resist divided by one-half of the loss in width

of metal immediately beneath the resist. Etch factors of 10 and higher are readily obtained by the method of the present invention and etch factors as high as 100 are not unusual.

The following examples are given to illustrate the present invention, but are not to be construed as limiting.

#### EXAMPLE 1

A magnesium photoengraving sheet having a nominal composition of 3 percent aluminum, 1.0 percent zinc, and minor alloying elements and impurities, balance magnesium, was photoprinted and developed in the conventional manner to prepare an acid resistant coating in the form of an image. A machine of the type described in U. S. Patent No. 2,669,048, was provided and approximately 3 liters of water at a temperature of about 60° F. placed therein. Thereafter, nitric acid of 42° Baumé technical was added to make a final concentration of  $\text{HNO}_3$  in the bath of 10 percent. Next, sufficient Monosulph (Nopco Chemical Company—a 45 percent sulfated castor oil) to make a 1.22 percent final solution mixed with sufficient diethyl-benzene to get a final concentration of 7 percent was added to the bath, and the volume adjusted with water to 5700 milliliters. The solution was mixed by running the paddles for two minutes. A photoengraving sheet, as above described, having the image thereon was descummed with an aqueous solution containing 12 ounces of potassium hydroxide and 4 ounces of potassium permanganate per gallon of solution. This plate was then placed in the plate holder of the machine, and the lid closed.

After the temperature of the bath had been brought to 72° F. by the heat exchanger, the paddles were started and adjusted to 500 R. P. M. and the etching continued for 8 minutes. There was thus obtained an average etch depth of .014-.015 inch with a smooth etched surface and a sharply delineated relief. The etch factor was 50.

#### EXAMPLE 2

In a manner similar to that of the above Example 1, except that zinc photoengraving plate having a nominal composition of 0.7 percent aluminum, and minor alloying elements, balance zinc, was substituted for the magnesium plate, the amount of Monosulph was reduced to 1.04 percent, the paddle speed was 600 R. P. M., and the time was 9 1/4 minutes. There was thus obtained an average etch depth of .019 inch having a smooth etched surface and a sharply delineated relief. The etch factor was 50.

#### EXAMPLE 3

In a manner similar to that of the foregoing Example 1, other half esters of sulfuric acid were substituted for the above Monosulph and the etching procedure repeated. The following table summarizes these results:

Table

| Trade name          | Sulfated                    | Principal Combined and Uncombined Fatty Acid Content                                                                 | Manufacturer         | Etch Factor Range | Concentration Percent Range Tested | Percent Optimum Concentration |
|---------------------|-----------------------------|----------------------------------------------------------------------------------------------------------------------|----------------------|-------------------|------------------------------------|-------------------------------|
| Turkey Red Oil..... | Castor OIL.....             | Ricinoleic Acid.....                                                                                                 | Nopco Chem. Co.....  | 2.6-100+          | 0.1-1.8                            | 1.0                           |
| Cordon 800/75.....  | do.....                     | do.....                                                                                                              | Finetex Inc.....     | 4.5-25            | 0.38-1.04                          | 0.90                          |
| Cordon 900.....     | Sperm OIL.....              | Stearic, Oleic, Linoleic, Palmitoleic, Arachidic, Palmitic, Myristic, Myristoleic, Lauric, and Behenic Acids.        | do.....              | 2.5-15            | 0.18-1.17                          | 1.0                           |
| Cordon LB870.....   | Tall Oils.....              | 50-60% $\text{C}_{10}-\text{C}_{18}$ Fatty Acids (primarily $\text{C}_{16}-\text{C}_{18}$ ) with 34-40% rosin acids. | do.....              | 6.2-15            | 0.38-0.81                          | 0.7                           |
| Drutone D.....      | Coconut and Olive Oils..... | Lauric, Myristic, Palmitic, Oleic, Linoleic, and Stearic Acids.                                                      | E. F. Drew & Co..... | 6-8               | 0.25-1.17                          | 1.1                           |
| Estol-T75.....      | Tallow.....                 | Myristic, Palmitic, Stearic, Oleic and Linoleic Acids.                                                               | do.....              | 8-14              | 0.25-1.17                          | 1.1                           |

In the above table, the Turkey red oil contained approximately 22 percent sulfation, while the others contained between 10 and 20 percent sulfation, depending on the amount of reaction products remaining with the desired material after purification by the supplier.

Each of the baths was relatively stable and each bath gave a very favorable etch when conditions were adjusted.

Various modifications may be made in the present invention without departing from the spirit or scope thereof, and it is to be understood that we limit ourselves only as defined in the appended claims.

We claim:

1. The method of etching the surface of an acid-soluble metal selected from the group consisting of magnesium, zinc, magnesium-base and zinc-base alloys said surface having portions thereof masked with an acid-resistant coating, which includes: repeatedly impinging upon the surface of the object so as to contact both the masked and unmasked portions thereof an aqueous solution which contains (1) from 1 to 25 percent of  $\text{HNO}_3$ , (2) a water-immiscible organic liquid substantially unreactive with the aqueous nitric acid, and (3) between 0.4 and 2.0 percent of a component which includes a water-soluble, anionic, sulfate-radical-containing, surface-active agent containing at least one hydrophobic group of from 10 to 26 carbon atoms in an uninterrupted chain and said agent containing at least 8 percent sulfation.
2. The method of etching the surface of an acid-soluble metal selected from the group consisting of magnesium, zinc, magnesium-base and zinc-base alloys, said surface having portions thereof masked with an acid-resistant coating, which includes: repeatedly impinging upon the surface of the object so as to contact both the masked and unmasked portions thereof an aqueous solution which contains (1) from 1 to 25 percent  $\text{HNO}_3$ , (2) a water-immiscible organic liquid substantially unreactive with the aqueous nitric acid, and (3) between 0.4 and 2.0 percent of a water-soluble, anionic, surface-active, sulfated, naturally-occurring oil containing at least 8 percent sulfation.
3. The method of claim 2 wherein the sulfated oil is castor oil containing about 45 percent sulfation.
4. The method of claim 2 wherein the organic oil is diethylbenzene.
5. The method of etching the surface of a magnesium plate having a portion of its surface masked with an acid-resistant coating, which includes: repeatedly impinging upon the surface of the plate so as to contact both the masked and unmasked portions thereof an aqueous solution which contains (1) 4 to 12.5 percent nitric acid, (2) 5 to 8 percent diethylbenzene, (3) and 1.16 percent sulfated castor oil having 45 percent sulfation.
6. An etching bath comprising an aqueous mixture of 1 to 25 percent  $\text{HNO}_3$ , from 1 to 12 percent of a water-immiscible organic liquid substantially unreactive with the aqueous nitric acid, and between 0.4 and 2.0 percent of a water-soluble, anionic, sulfate-radical-containing surface-active agent containing at least one hydrophobic

group of from 10 to 26 carbon atoms in an uninterrupted chain, said agent containing at least 8 percent sulfation.

7. An etching bath comprising a mixture of 1 to 25 percent nitric acid, a water-immiscible organic liquid sub-

stantially unreactive with the aqueous nitric acid, and between 0.4 and 2.0 percent of a water-soluble, anionic, surface-active, sulfated, naturally-occurring oil containing at least 8 percent sulfation.

8. The bath of claim 7 wherein the sulfated oil is 5 castor oil containing about 45 percent sulfation.

9. The bath of claim 7 wherein the organic liquid is diethylbenzene.

10. An etching bath comprising a mixture 4-12.5 percent nitric acid, 7 percent diethylbenzene, and 1.16 percent sulfated castor oil having 45 percent sulfation. 10

References Cited in the file of this patent

UNITED STATES PATENTS

2,640,765 Easley et al. ----- June 2, 1953

OTHER REFERENCES

Schwartz-Perry: Surface Active Agents, publ. 1949, Interscience Pub. Inc., N. Y., p. 462, lines 7-11.